

## UNITED STATES PATENT OFFICE

2,649,361

METHOD OF DISSOLVING METALS AND  
COMPOSITION THEREFOR

Richard Springer, Leipzig, Germany, and Walter R. Meyer, Hamden, Conn., assignors to Enthone, Incorporated, New Haven, Conn., a corporation of Connecticut

No Drawing. Application December 24, 1949, Serial No. 135,037. In Germany May 13, 1949

14 Claims. (Cl. 41—42)

1

This invention concerns dissolving metals of the class consisting of nickel, copper, cadmium, silver, zinc, and gold, by chemical action alone, that is to say, without the aid of an electric current, and especially to stripping such metals, that is, reducing the thickness of walls of articles made of metals of the foregoing list and removing more or less completely electroplates and other coatings of such metals formed on foundations of other materials.

The invention involves a process, baths suitable for use with the process, and compositions of matter from which such baths can be made readily.

Heretofore it has been proposed to strip unsatisfactory coatings, e. g. poorly done, incomplete, or damaged electroplates, from their basis or foundation metals by immersing the articles in an acid bath, e. g. a sulfuric acid bath, and with or without the aid of an electric current. Commonly at least however, with such prior procedures, the basis or foundation metal is attacked when and where exposed to the bath. Further, it has been known for some time that solutions of cyanides will dissolve certain metals in the presence of air. It has been known also that the addition of certain inorganic oxidizing agents of high oxidizing potentials to cyanide solutions, causes the cyanide solutions to dissolve these metals at rates greater than when such agents are absent. These agents render the solutions unstable however, so that the solutions tend to break down rapidly, and in some instances the agents render the solutions explosive.

In contrast with this, speaking generally, we have discovered that aqueous solutions containing both one or more of the cyanides hereinafter identified, and one or more nitro-substituted aromatic compounds of the class hereafter defined, are capable of dissolving the metals of the class consisting of nickel, copper, cadmium, zinc, silver and gold, at rates which are, respectively, greater than the rates of dissolution of those metals in solutions of cyanide alone in corresponding concentrations, and at the same time without the unsatisfactory accompanying characteristics of the prior practices, i. e. without a too rapid breakdown of the bath or solution, at least with properly chosen proportions, without tendency of the bath to breakdown with explosive violence, and commonly at least, by a proper selection of materials, without substantial attack on ferrous foundation or basis materials that may underlie the metal to be dissolved. The cyanides are ammonium cyanide and those alkali metal cyanides

2

and those alkaline earth cyanides which are ionizable in water to give cyanide ions and soluble in water to such an extent that at least 2.5 grams of the cyanide radical can be dissolved per liter of the solution, at least at the temperature at which the present process is used. For conciseness all the cyanides thus identified are referred to herein as the alkali cyanides. The nitro-substituted aromatic compounds are those nitro-substituted aromatic compounds which, in solution in water, produce an electromotive force of minus 0.9 volt, or a higher voltage than this, between a sheet nickel electrode and a saturated potassium chloride calomel electrode under the following conditions: the concentration of the nitro-compound is its saturation value or is about 0.25 gram-mol per liter of the solution, whichever is the smaller; there is present in the solution 2 gram-mols of sodium cyanide per liter of solution; if the nitro-compound is an acid or otherwise tends to cause an evolution of hydrocyanic gas, there is added also sufficient sodium hydroxide to neutralize, or to render the solution sufficiently alkaline to substantially prevent the evolution of hydrocyanic gas; the temperature is 80° C. ± 1° C. For example, a solution of o-nitrochlorobenzene produces under such conditions (the solution being saturated as to this nitro-compound, and no sodium hydroxide being present), a voltage of minus 0.9 volt. Again, a solution of m-nitrobenzoic acid produces under the prescribed conditions (the concentration of the acid being 42 grams per liter of the solution and 10 grams per liter of sodium hydroxide being added, substantially enough to neutralize the acid to its sodium salt), a voltage of about minus 0.66 volt, i. e. a voltage higher than that of the o-nitrochlorobenzene. Wherever hereinafter a voltage producible by a nitro-compound is referred to, it is to be understood to be a voltage producible between a sheet nickel electrode and a saturated potassium chloride calomel electrode under the foregoing conditions.

Speaking generally, the present process consists of subjecting the metal or metals to be dissolved to an aqueous solution of one or more such cyanides and one or more such nitro-substituted aromatic compounds, at a temperature or various temperatures between room temperature or even somewhat lower and the boiling point of the solution, until the desired dissolution of the metal has been achieved. Speaking generally, the higher the temperature at which the operations are carried out, the higher the rate of dissolution of the metal. However, the higher the temperature the

more rapidly the solution deteriorates also. Usually a temperature between about 70° C. and about 95° C. is used; usually about 80° C. is preferred for general operations. The quantity of cyanide or cyanides used in any instance can be anywhere from that quantity which provides about 2.5 grams of the cyanide radical per liter of the solution, to sufficient to saturate the solution. However there seems to be an optimum quantity for the cyanide radical, i. e. a quantity at which the effect of the cyanide content is at a maximum, namely between about 13 grams per liter and about 105 grams per liter; usually about 52 grams per liter to about 86 grams per liter of cyanide radical, more or less, is suitable for general purposes. The quantity of the nitro-compound or nitro-compounds used in the solution can be anywhere from that quantity which will provide between about 0.155 gram of the nitro-benzo grouping, i. e.



per liter of solution and sufficient to saturate the solution with the nitro-compound or nitro-compounds. Speaking generally, the greater the quantity of the nitro-benzo group present, the higher is the rate at which the metal is dissolved. About 32 grams of the nitro-benzo group per liter of the solution gives a sufficiently high rate for general purposes usually, although at times 52 grams, or even 70 grams, per liter and the correspondingly higher rate of metal dissolution is desirable in practice. As between the nitro-benzo grouping and the cyanide radical, the quantity of the nitro-benzo grouping can be from as low as one-tenth of one percent of the quantity of the cyanide radical to a very much higher figure; theoretically, apparently, to some hundreds percent. Generally however between about 30% and about 150% is used, and between about 55% and about 90% (i. e. the quantity of the nitro-benzo grouping being between about 55% and about 90% of the quantity of the cyanide radical used) seems to be satisfactory, for most general purposes at least. When the nitro-compound used in making up the metal-dissolving solution is an acid (as, of course, it may or may not be), or where the compound is one that tends to act as an acid, causing evolution of hydrocyanic gas, the solution can be neutralized, e. g. by the addition of an alkali as will be understood, or at least the solution made sufficiently alkaline to prevent substantial evolution of hydrocyanic gas. For example, a solution in water of m-nitrobenzoic acid, 45.5 grams per liter of solution, sodium cyanide, 100 grams per liter, and sodium hydroxide, 10.8 grams per liter to neutralize, is quite a satisfactory solution. However the addition of alkali to an extent noticeably greater than that required to neutralize the solution does not inhibit the metal-dissolving action of the solution, at least to a material extent. As an example, a water solution of m-nitrobenzoic acid, 100 grams per liter of solution, potassium cyanide, 200 grams per liter, and potassium hydroxide, 50 grams per liter (the latter being about 50% more than is required to neutralize the acid), also dissolves, say, nickel at a generally satisfactory rate. In some instances, particularly where the metal is to be dissolved to a considerable depth (say to a depth of more than 0.001

inch or something of that order), or where some certain nitro-compounds are used, the rate of dissolution of the metal from a given piece, while starting initially and continuing for a time at relatively high values, may fall later to an undesirably lower value, due either, say, to a tendency to passivity or to the formation of a foreign deposit on the metal surface; in such instances the articles can be removed from the solution and rinsed with water (e. g. until any deposit on the surface is removed) and then returned to the solution; this raises the rate of dissolution again. Also in some instances agitation, i. e. movement of the solution over the surface to be dissolved or movement of the article in the solution, raises the rate of dissolution of the metal very materially, whether by preventing the deposition of reaction products on the metal surface or otherwise; an increase in the rate of metal dissolution of as high as 40% by agitation has been observed; in some instances agitation has not seemed to hasten the dissolution however. After a required amount of the metal has been removed from an article, the article may be rinsed thoroughly in clean water to stop the action. Rinsing in an acidic rinse should be avoided unless precautions are taken, since such a rinse may cause the evolution of toxic hydrocyanic gas.

The solution deteriorates both with age and with use. After the rate of dissolution has fallen materially because of consumption of the solute, or because of dragout, the solution can be replenished, generally at least twice if the solution is used continuously from the start, say by the addition of cyanide and the nitro-compound, with or without neutralizing alkali, and say in the same proportions of these, one to the other, as in the initial solution. Subsequently however the solution deteriorates to such an extent and in such a way that it is better to discard the solution and make up a new one; this is indicated when the rate of dissolution of the metal falls to an undesirably low value and fails to rise again adequately on further replenishment.

Before the operation is begun the surface of the metal to be dissolved should be cleaned thoroughly of course, say with an alkali cleaner to remove organic dirt, and with acids to remove passive films if any are present.

As an example of the process: Take for each liter of solution to be prepared, 45.5 grams of m-nitrobenzoic acid, 10.8 grams of sodium hydroxide, and 100 grams of sodium cyanide, and dissolve them in sufficient water to make up the desired quantity of solution. To hasten complete solution of these materials, the water can be heated to, say, 75° C. and the quantity of solution measured at this temperature. However the quantities of the solids per liter of solution can be varied so widely, as appears from the foregoing, that the temperature at which these proportions are determined is not of great importance. Heat this solution or bath to about 80° C., and while holding it at this temperature hang in it plates of cold rolled steel electroplated with nickel. Speaking generally, each plate is held in the bath until the whole of the nickel plate, or such a thickness of the plate as desired, has been dissolved away. However if the stripping action ceases on a particular plate before the nickel has been dissolved to the desired depth, remove the piece from the solution and rinse it in clean non-acidic running water, removing any deposit or residue that may be on it, and then return the piece to the metal-dissolving bath. Dissolution

at this piece then begins again, unless, of course, the bath is deteriorated too much. When the desired amount of nickel has been removed from any piece, remove the piece and rinse it thoroughly in clean non-acidic running water. As one or more pieces are finished they may be replaced by new work for similar treatment. As the rate of metal dissolution falls due to dragout or consumption of the solute during the first eight hours of continuous use, add water to the bath as necessary and also add further of the nitro-compound, hydroxide and cyanide to the bath in about the same proportions to each other as initially. This more or less restores the dissolution rate. Usually additions of the nitro-compound, hydroxide and cyanide amounting to as much as 75% of the quantity of those materials with which the bath was made up initially, can be made to the bath during the first day. The dissolution rate is high for about the first eight hours use usually, and then falls gradually so that the second day the rate is noticeably lower than during the first day. The bath can be replenished again the second day, but after, say, the third successive day of use the bath will have deteriorated to such a degree that it is well to discard it and make up a fresh bath for further work. Most low carbon steels, cold rolled steels and cast irons are not attacked by such a bath when freshly made; accordingly when the foundation or basis metal underlying the nickel plate is formed by any of these, the foundation or basis of the nickel, wherever it may be exposed to the bath, is not affected by the nickel stripping operation; if after some use of the bath such a foundation is attacked, this indicates that the bath has deteriorated and should be discarded. However, some types of high carbon steels and cast irons are attacked slightly by solutions or baths made up as here described. During the metal-dissolving operation a small amount of cyanide fumes is given off, i. e. to about the same extent as with a hot cyanide plating solution, and in addition an odor of ammonia. Accordingly exhaust ventilation should be provided for the tank in which the solution is held.

As other examples: Take the same acid, hydroxide and cyanide as in the first example, but using per liter of solution 20% more than the quantity of each stated in that example. With the same operations, the results are substantially the same as before but the rate of dissolution of the nickel is higher than in the first example. Again, take the same solutes as before but use per liter of solution 75% more than the quantity of each stated in the first example. With substantially the same operations as before, the results are substantially the same except the nickel is dissolved at a still higher rate.

As still another example: For each liter of solution to be prepared, take 51.5 grams of m-sodium nitro-benzoate and 100 grams of sodium cyanide and dissolve them in sufficient water to make up the desired quantity of solution. The procedure and operations of the first example can be followed and substantially the same results obtained.

With such solutions or baths and operations as those just described, electroplated nickel is dissolved at rates of from about 0.0005 to 0.002 or more inch per hour (i. e. is reduced in thickness at such rates when the bath is acting on one side only of the plate), the rate in any instance depending primarily on the concentration of the solutes in the bath, the temperature

of the operations, the age of the bath and the extent to which the bath has been used, and perhaps the process by which the nickel is electroplated.

As a still further example: Make up the bath containing m-nitrobenzoic acid, potassium cyanide and potassium hydroxide which is described above, heat it to 80° C., and while holding at this temperature hang plates of electroplated nickel in it. The nickel is dissolved at rates even higher than those mentioned above.

Nitrobenzoic acid together with sufficient hydroxide to neutralize or an excess of the hydroxide, or equivalently a nitrobenzoate salt such as results from the reaction between such acid and hydroxide, seem to be preferable to the other nitro-compounds, because of the wide range of stripping rates which can be obtained by using smaller or larger quantities of them per liter of water. The meta form seems to be especially preferable for general use since not only does it have a wide range of stripping rates but also it is generally available and it tends to have stripping rate greater than that of the para form even. For example, under like conditions the meta form has given a stripping rate of 0.00216 inch of nickel per hour while the para form gave a rate of 0.00149 inch per hour.

However, other nitro-compounds are useable as appears from the foregoing. For example, and for the purposes of comparison: (The following figures of this paragraph were obtained from aqueous solutions containing 98 grams of sodium cyanide per liter of solution, operation at 80° C., the grams per liter stated are grams of the respective substances per liter of the solution, "sat. sol." indicates that the bath or solution was saturated with the respective compound, and the "rate" figures indicate substantially the initial stripping rates of electroplated nickel in fractions of an inch per hour.) Nitroanilines; e. g. o-nitroaniline, sat. sol., voltage minus 0.82, rate 0.00013; again, m-nitroaniline, sat. sol., voltage minus 0.73, rate 0.000598; and again, p-nitroaniline, sat. sol., voltage minus 0.81, rate 0.00018. Nitrophenols, e. g., o-nitrophenol, 35 grams per liter, sodium hydroxide 10 grams per liter, voltage minus 0.83, rate 0.00014; again, 2-nitroresorcinol, 39 grams per liter, sodium hydroxide 10 grams per liter, voltage minus 0.76, rate 0.000320; and again, 2,4-dinitroresorcinol, 25 grams per liter, sodium hydroxide 10 grams per liter, voltage minus 0.78, rate 0.000182; still again, 2,4,6-trinitroresorcinol, 21 grams per liter, sodium hydroxide 10 grams per liter, voltage minus 0.76, rate 0.000235. Nitrobenzene sulfonic acid; e. g. m-nitrobenzene sulfonic acid, 57 grams per liter, sodium hydroxide 10 grams per liter, voltage minus 0.65, rate 0.00242. Nitrobenzaldehydes; e. g. m-nitrobenzaldehyde, 38 grams per liter, voltage minus 0.70, rate 0.00062. Also p-nitrotoluene, o-nitrochlorobenzene, and p-nitrochlorobenzene are useable, but they are of rather low solubilities, their voltages are rather low, and their stripping rates are relatively low. Incidentally the m-nitrobenzene sulfonic acid seems to tend to rather considerable self-decomposition, and with m-nitrobenzaldehyde an orange colored precipitate has been noticed.

The foregoing specific matters have been devoted to the action on nickel so that the results obtainable with the various materials can be compared. As appears earlier above however, the same process is applicable to stripping copper,

zinc, cadmium, gold and silver also. For example, an aqueous solution containing 98 grams per liter of sodium cyanide and 10 grams per liter of m-sodium nitrobenzoate, at 80° C., stripped the following metals, electroplated from standard cyanide solutions, at the following rates in inch per hour: silver, 0.000193; copper, 0.00173; cadmium, 0.00157; zinc, 0.00105; and when the benzoate concentration was 47 grams per liter: silver, 0.00525; copper, 0.00783; cadmium, 0.00766; zinc, 0.00746.

Speaking generally at least, one or more of the cyanides identified above and one or more of the nitro-compounds can be mixed in the dry state in appropriate proportions for baths for the present process, and stored and transported in this form for use when and where needed. The proportions are those appearing above of course where necessary to neutralize or prevent evolution of gas from the solution, one or more hydroxides can be included in the dry mixtures.

It will be understood that the invention is not limited to the details of materials and operation mentioned above, except as appears hereafter in the claims, and that the claims are intended to include equivalents of the various matters appearing in them as well as those matters specifically.

We claim:

1. A metal-dissolving composition for dissolving metals by chemical action containing at least one water-soluble alkali cyanide that is ionizable in water to the extent to yield at least 2.5 grams of cyanide radical per liter of aqueous solution, and at least one nitro-substituted aromatic compound capable of producing an electrical potential of minus 0.9 volt or higher between a sheet nickel electrode and a saturated potassium chloride calomel electrode, the nitro benzo grouping of the nitro-compound being, by weight, equal to more than one-tenth of one percent of the cyanide radical, and the composition being alkaline in reaction and being substantially free from nickel, copper, cadmium, silver, zinc and gold.

2. A metal-dissolving composition for dissolving metals by chemical action containing at least one water-soluble alkali cyanide that is ionizable in water to the extent to yield at least 2.5 grams of cyanide radical per liter of aqueous solution, and at least one nitro-substituted aromatic compound capable of producing an electrical potential of minus 0.9 volt or higher between a sheet nickel electrode and a saturated potassium chloride calomel electrode, the nitro benzo grouping of the nitro-compound being, by weight, equal to between about 30% and about 150% of the quantity of the cyanide radical, and the composition being alkaline and substantially free from nickel, copper, cadmium, silver, zinc and gold.

3. The subject matter of claim 1 characterized by the fact that the nitro-compound content consists of at least one material selected from the group consisting of nitrobenzoic acid, nitroaniline, nitrophenol, nitrobenzene sulfonic acid, nitrobenzaldehydes, and neutralized forms of any of the foregoing.

4. The subject matter of claim 1 characterized by the fact that the alkali cyanide is an alkali metal cyanide, the aromatic compound is a nitrobenzoic acid, and at least one hydroxide is included in the composition.

5. The subject matter of claim 1 characterized

by the fact that the cyanide is an alkali metal cyanide and the aromatic compound is m-nitrobenzoate.

6. A metal-dissolving solution of water, at least one alkali cyanide that is ionizable in water to the extent to yield at least 2.5 grams of cyanide radical per liter of solution, the quantity of the cyanide being sufficient to provide the metal-dissolving solution with at least 2.5 grams of cyanide radical per liter of the solution, and at least one nitro-substituted aromatic compound capable of producing an electrical potential of minus 0.9 volt or higher between a sheet nickel electrode and a saturated potassium chloride calomel electrode, the quantity of said aromatic compound being sufficient to provide the solution with at least 0.155 gram of the nitro-benzo grouping per liter of solution, and the solution being substantially free from nickel, copper, cadmium, silver, zinc and gold.

7. The method of dissolving away an exposed surface of a metal of the class consisting of nickel, copper, cadmium, silver, zinc and gold, which consists in subjecting the surface to an aqueous solution containing per liter of solution, at least about 2.5 grams of cyanide radical and at least about 0.155 gram of nitro-benzo grouping of a nitro-substituted aromatic compound capable of producing an electromotive force of at least minus 0.9 volt between a sheet nickel electrode and a saturated potassium chloride calomel electrode, in the absence of a substantial flow of electric current between said surface and the solution.

8. The subject matter of claim 7 characterized by the fact that the solution is held at a temperature between about 70° C. and about 95° C.

9. The method of dissolving away an exposed surface of a metal of the class consisting of nickel, copper, cadmium, silver, zinc and gold, which consists in subjecting the surface to an aqueous solution containing, per liter of solution, between about 13 grams and about 105 grams of cyanide radical and more than 0.155 gram of nitro-benzo grouping of a nitro-substituted aromatic compound capable of producing an electromotive force of at least minus 0.9 volt between a sheet nickel electrode and a saturated potassium chloride calomel electrode, in the absence of a substantial flow of electric current between said surface and the solution.

10. The subject matter of claim 9, characterized by the fact that the solution contains between about 52 grams and 86 grams of cyanide radical per liter of solution and the solution is alkaline.

11. The subject matter of claim 10 characterized by the fact that by weight the quantity of the nitrobenzo grouping is between about 30% and 150% of the cyanide radical.

12. The method of dissolving away an exposed surface of a metal of the class consisting of nickel, copper, cadmium, silver, zinc and gold, which consists in subjecting the surface to an aqueous solution of at least one alkali cyanide, at least 5 grams per liter of solution, and at least one nitro-substituted aromatic compound, at least 2.2 grams per liter of solution, selected from the following: nitrobenzoic acid, nitroaniline, nitrophenol, nitrobenzene sulfonic acid, nitrobenzaldehydes, and neutralized forms of any of the foregoing.

13. The subject matter of claim 12 characterized by the fact that the solution is alkaline.

14. The method of dissolving away an exposed

## 9

surface of a metal of the class consisting of nickel, copper, cadmium, silver, zinc and gold, by chemical action, which consists of subjecting the surface to an aqueous solution of at least one alkali cyanide, sufficient to provide between about 52 grams to 86 grams of cyanide radical per liter of solution, and at least one alkali m-nitrobenzoate, sufficient to provide between about 52 grams and about 70 grams of nitro-benzo grouping per liter of solution.

RICHARD SPRINGER.  
WALTER R. MEYER.

References Cited in the file of this patent

## UNITED STATES PATENTS

## 10

Number  
585,854  
859,482  
2,059,052  
5 2,085,776  
2,287,654  
2,428,464  
2,435,889

Number  
813  
391,468

## 15

Number Name Date  
331,810 Mutchler Dec. 8, 1885

## 10

| Name     | Date          |
|----------|---------------|
| Sully    | July 6, 1897  |
| Bueb     | July 9, 1907  |
| Sperr    | Oct. 27, 1936 |
| Vaughen  | July 6, 1937  |
| Wernlund | June 23, 1942 |
| Lum      | Oct. 7, 1947  |
| Kerridge | Feb. 10, 1948 |

## FOREIGN PATENTS

| Country       | Date          |
|---------------|---------------|
| Great Britain | June 18, 1903 |
| France        | Aug. 31, 1908 |